

W. T. SCHREIBER.

PROCESS OF PRODUCING LIQUID FUELS.

APPLICATION FILED JAN. 31, 1918.

1,405,805.

Patented Feb. 7, 1922.



INVENTOR  
Walter T. Schreiber,  
Prudde, Wright & Small.  
ATTORNEY

# UNITED STATES PATENT OFFICE.

WALTER T. SCHREIBER, OF BALTIMORE, MARYLAND, ASSIGNOR TO U. S. INDUSTRIAL  
ALCOHOL CO., A CORPORATION OF WEST VIRGINIA.

## PROCESS OF PRODUCING LIQUID FUELS.

1,405,805.

Specification of Letters Patent. Patented Feb. 7, 1922.

Application filed January 31, 1918. Serial No. 214,753.

*To all whom it may concern:*

Be it known that I, WALTER T. SCHREIBER, of Baltimore, in the State of Maryland, have invented a certain new and useful Improvement in Processes of Producing Liquid Fuels, and do hereby declare that the following is a full, clear, and exact description thereof.

My invention relates particularly to processes for making fuels designed to be used in any desired manner, but it has application especially to processes for making fuels adapted to be used as a source of power, as for example fuels for burners and motor fuels.

The object of my invention is to provide processes for making a fuel containing a light hydrocarbon, as well as alcohol and an ingredient adapted to blend the same or to form a solution with the hydrocarbon and alcohol.

A further object of my invention is to provide processes for making a fuel of this character which is of such a nature that only a very small quantity of the third ingredient is found necessary.

A further object is to provide processes for making a fuel of this character which contains a large percentage of the light hydrocarbon, notwithstanding the small percentage of the third ingredient.

A further object of my invention is to provide processes for making a fuel of this character in which the third ingredient is acetylene.

A further object of my invention is to provide processes for making a fuel of this character which contains dehydrated alcohol or absolute alcohol.

A further object of my invention is to provide an advantageous process for dehydrating the alcohol.

Further objects of my invention will appear from the detailed description thereof contained hereinafter.

While my invention is capable of being carried out in many different ways, for the purpose of illustration I shall describe only certain ways of carrying out the same herein. Furthermore, while my invention is capable of being carried out in connection with many different types of apparatus, I have shown only one type of apparatus for use

in connection with the same in the accompanying drawings, in which— 55

The figure is a diagrammatic representation of an apparatus which may be used in connection with my invention.

For example, a fuel made in accordance with my invention may be made as follows: 60 50 c. c. of ethyl alcohol, having a strength of 95%, is added to an excess of calcium carbide, amounting usually to 10 grams, in a container 1, having a valved inlet opening 2 and a valved outlet pipe 3. The calcium carbide is acted upon by the water in the alcohol so as to produce acetylene, a portion of which dissolves in the alcohol while the balance is carried off by a tube 4, connected to the top of the container 1, and is then 70 passed into a mixture of 50 c. c. of gasoline and 40 c. c. of kerosene in a vessel 5, so arranged that the end of the tube 4 extends down into the body of liquid therein, and having a valved outlet pipe 6. The contents of the container 1 are then removed from the same by means of the valved outlet 3 located in the bottom of the container, and the calcium hydroxide and any undecomposed calcium carbide is filtered off 80 from the liquid, which is a dehydrated alcohol having a strength of approximately 99%; and containing approximately 1% of acetylene dissolved therein,—that is to say, a saturated solution of acetylene.

The alcohol thus produced is then mixed with the mixture of gasoline and kerosene, containing acetylene obtained as above, thus providing a fuel oil that remains homogeneous and which is advantageous for use as a 90 motor fuel or for burners.

Another composition containing the dehydrated alcohol may be comprised of 50 c. c. of the alcohol dehydrated as before, 50 c. c. of gasoline and 40 c. c. of kerosene 95 to which no acetylene has been added.

As another mode of procedure in producing fuels in accordance with my invention, I may begin as follows: 100 50 c. c. of ethyl alcohol, which may have been previously partially dehydrated or not, as desired, mixed with 50 c. c. of gasoline and 40 c. c. of kerosene, are introduced into the container 1, and an excess of calcium carbide, usually amounting to 10 grams, is then added thereto. The mixture is then allowed to 105

stand for one or more days, until eventually all of the acetylene produced dissolves in the mixture. The contents of the container 1 are then drawn off by the pipe 3 and filtered, so as to remove the calcium hydroxide and any undecomposed calcium carbide, thus leaving a homogeneous mixture containing dehydrated alcohol, gasoline and kerosene containing approximately 1% of acetylene.

Furthermore, in either of the above examples, if it is desired to add more acetylene, this may be done by adding thereto 15 c. c. of acetone saturated with acetylene.

15. The dehydration of the alcohol very materially assists in the blending of the same with the gasoline and kerosene and the acetylene contained in the mixture also assists, to some extent, in accomplishing the same end.

20. The addition of the acetylene to the fuel, furthermore, assists in improving the character of the fuel by increasing its explosibility. This is especially advantageous where the fuel is to be used as a motor fuel. Where

25 acetone is added, this also has a similar effect in increasing the readiness with which the mixture explodes when used as a fuel.

It will be understood that the dehydrated alcohol need not necessarily be of the 30 strength above referred to, but may be of any strength above the 95% strength obtained commercially.

It will be understood, however, that, instead of the gasoline and kerosene referred 35 to in the above examples, I may use only gasoline.

While I have described my invention above in detail, I wish it to be understood that many changes may be made therein without 40 departing from the spirit thereof.

I claim:

1. The process which comprises dehydrat-

ing ethyl alcohol with a carbide, then collecting the evolved gaseous hydrocarbon in a quantity of gasoline and kerosene, and adding the alcohol to the gasoline and kerosene containing the absorbed hydrocarbon.

2. The process which comprises dehydrating ethyl alcohol with calcium carbide and absorbing some of the acetylene evolved 50 therein, collecting the acetylene not so absorbed in a quantity of gasoline and kerosene, and adding the latter to the alcohol.

3. The process which comprises making a fuel consisting of alcohol, a light hydrocarbon oil resulting from petroleum distillation, and a heavier hydrocarbon, involving adding a carbide to dehydrate the alcohol and allowing the acetylene formed to dissolve therein, whereby a suitable composition is formed 60 which will not separate into its constituents at low temperatures.

4. The process of manufacturing a fuel comprising dehydrating alcohol with a carbide, passing acetylene generated into a light 65 hydrocarbon oil, and mixing the latter with the alcohol.

5. The process which comprises making a fuel comprising alcohol, a light hydrocarbon oil resulting from petroleum distillation, and 70 a heavier hydrocarbon oil, the proportion of the hydrocarbon oils being greater than that of the alcohol, involving the step of treating the alcohol with a carbide to dehydrate it, and allowing the acetylene generated to dissolve in the mixture, whereby a suitable composition is formed which will not separate at low temperatures.

In testimony that I claim the foregoing I have hereunto set my hand.

WALTER T. SCHREIBER.

Witnesses:

ARTHUR A. BACKHAUS,  
ERNEST J. WINTER.